# EUROPEAN PATENT APPLICATION

(11) **EP 4 403 682 A1**
(43) Date of publication of application: **24.07.2024**
(21) Application number: 23152852.2
(22) Date of filing: 23.01.2023
(51) Int. Cl.: D02G 3/36

(54) **COVERED SHAPE-MEMORY POLYMERIC FIBERS FOR TEXTILE APPLICATIONS**

(71) Applicant: Helmholtz-Zentrum hereon GmbH, 21502 Geesthacht (DE)
(72) Inventor: Izraylit, Victor, 10179 Berlin (DE); Farhan, Muhammad, 12279 Berlin (DE)
(74) Representative: Uexküll & Stolberg

(57) **Abstract**

The present invention relates to the field of textiles, in particular shape-memory polymeric fibers (SMPF) for textile applications or medical applications where shape fixity and recovery can be kept constant over multiple shape-memory cycles. The present invention provides a covered shape-memory polymeric fiber having a core fiber of semi-crystalline polymer and a substantially unstretchable covering yarn wound around the core fiber in a manner that the maximum engineering strain (εₘₐₓ) of the core shape-memory fiber is reduced to at most the strain at the yield point (ε_{yield}) of the uncovered core fiber. Thus, the covering yarn is used to limit the stretchability or deformation of the core shape-memory fiber during programming so as to ensure maximum recoverable strain.

## Description

The present invention relates to the field of textiles, in particular shape-memory polymeric fibers and was partly developed under the EU project "GrowBot - Towards a new generation of plant-inspired growing artefacts" (Grant Agreement 824074).

### BACKGROUND OF THE INVENTION

Shape-Memory Polymers (SMPs) are an emerging class of smart materials which are able to modify their size and shape in response to external stimuli such as heat, electric and magnetic field, water or light. Typical SMPs have the ability to memorize their original shape after deformation such as stretching. They maintain the deformed state in the absence of the stimulus, and recover their original shape after application of the external stimulus. SMPs have been increasingly investigated for biomedical applications. From a structural view point, SMPs can be classified as three-dimensional systems, such as shape memory blocks or shape memory foams, two-dimensional systems, such as shape memory films, and one-dimensional systems such as shape memory fibers, where shape memory fibers have drawn the most attention. In a woven form shape memory fibers can be converted into two-dimensional and/or three-dimensional systems.

SMPs in the form of fibers are generating great interest in structural and functional applications because of their flexibility, anisotropic properties and their capability of being converted into two-dimensional and/or three-dimensional systems. Known shape memory fibers have been produced from polyurethane block copolymers or from multiblock copolymers comprising poly(ω-pentadecalactone) hard segments (PPDL) and poly(ε-caprolactone) switching segments (PCL) via electrospinning methods as disclosed in F. Zhang et al. "Shape memory polymer nanofibers and their composites: electrospinning , structure, performance, and applications" Frontiers in Materials, October 2015, Vol. 2, Article 62, or from poly(ethylene-co-vinyl acetate) random copolymers, as disclosed in K. Wang et al. "The Thermal and Mechanical Properties of Poly(ethylene-co-vinyl acetate) Random Copolymers (PEVA) and its Covalently Crosslinked Analogues (cPEVA)", Polymers 2019, 11, pages 1055 (2019) via extrusion.

Chinese patent application CN 1706997 A discloses a shape memory fiber prepared from shape memory polyurethane and its preparation method and Chinese utility model CN 201553838 U discloses a heat-sensitive shape memory polyurethane covered yarn (shape-memory polymeric fibers, cSMPF) and a method of producing it.

Said cSMPF can be programmed by stretching at various temperatures before or after covering with conventional yarns in textile industry such cotton, nylon, and polyester etc. Compared with the covered yarn structure of other fibers, the thermosensitive shape memory polyurethane disclosed here had stronger fabric wrinkling prevention capability with better elasticity and was easy to be recovered to permanent initial shape.

This covering is not only necessary to overcome the processing related technical constraints, but also they are sometime necessary for comfort and due to regulatory requirements where the direct contact of such fibers to the body of the wearer can be avoided. Compared with the covered yarn structure of other fibers, the thermosensitive shape memory polyurethane disclosed in CN 201553838 U is stated to have improved fabric wrinkling prevention capability and improved elasticity. The diameter ratio between the covering yarn and core yarn is reported as ranging from 0.1 to 1.0.

WO 2012/045427 A1 discloses medical aids, in particular body support bandages and orthotics, comprising at least one element which generates or delivers a supporting force, compression or introduction of pressure, and which comprises shape memory material or consists thereof. The programmed shape memory transition of the medical aid is triggered by body heat whereby the stretched form of the medical aid, which facilitates application to the body, changes into a contracted form conveying the supporting and/or compression effect of the medical aid. The shape memory material according to this disclosure is a composite material, a mixture, an alloy, or a composite material having different shape memory effects.

In textile industry there is still a need for products with shape-memory properties which should be useful in particular for medical applications. In particular there is still a need for shape-memory polymeric fibers (SMPF) for textile and/or medical applications where shape fixity and recovery can be kept constant over multiple shape-memory cycles.

### SUMMARY OF THE IVENTION

In one aspect, the present invention relates to a covered shape-memory polymeric fiber (cSMPF) having a core fiber of semi-crystalline polymer fibers and a substantially unstretchable covering yarn wound around the core fiber in a manner that the maximum engineering strain (εₘₐₓ) of the core shape-memory fiber is reduced to at most the strain at the yield point (ε_{yield}) of the uncovered core fiber. Thus, the covering yarn is used to limit the stretchability or deformation of the core shape-memory fibers during programming so as to ensure maximum recoverable strain. The maximum deformation of the core fiber of a given length (L₀) and diameter (D₀) in the unstretched state by covering the fiber with a covering yarn can be influenced by the density of entwining (ρ₀) of the core fiber in the unstretched state, i.e. by the number of twists per meter of the covering yarn when the core fiber is in the unstretched state, and the length (l) and diameter (d) of the covering yarn, all in relation to the diameter of the core fiber (D₀) in the unstretched state.

Upon applying a stress to the covered fiber so as to stretch the fiber, the length (L₁) of the core fiber increases, whereas the density of entwining (ρ₁) decreases. The strain (ε) of the core fiber is given by the following formula: ${ε}_{1} = \frac{{L}_{1} - {L}_{0}}{{L}_{0}} \times 100 % ,$ wherein ε₁ is the strain, L₁ is the length of the core fiber at said stress, L₀ is the length of the core fiber in the unstretched state.

Stretching (elongation) of the core fiber having the covering yarn wound around it causes the pitch (r), i.e. the distance between two loops of the twist, of the covering yarn around the core fiber to increase from r₀ to r₁, whereby the density of entwining (ρ₁) decreases. The covering yarn is not stretched until up to a maximum strain (εₘₐₓ) of the core fiber. Further stretching of the core fiber beyond the maximum strain (εₘₐₓ) would require stretching of the covering yarn as well. Under the premise that the covering yarn is substantially unstretchable, stretching the fiber beyond the point of maximum strain (εₘₐₓ) would cause rupture of covering yarn.

According to the present invention, this point of maximum strain (εₘₐₓ) of the core fiber should be chosen so as to not exceed the strain at the yield point (ε_{yield}) of the core fiber. The point of maximum strain (εₘₐₓ) is independent of the material of the covering yarn, and solely dependent on the diameter (D₀) of the shape-memory polymeric core fiber (cSMPF), the diameter of the covering yarn (d) and the density of entwining (ρ₀), wherein the density of entwining (ρ₀) is defined as: ${ρ}_{0} = \frac{{n}_{0}}{{L}_{0}} ,$ wherein ρ₀ is the density of entwining, L₀ is the length of the core fiber in the unstretched state and n₀ is the number of windings of the covering yarn around the core fiber in the unstretched state.

The length of the covering yarn, dependent on the length of the core fiber, required to achieve that the maximum engineering strain (εₘₐₓ) of the core shape-memory fiber is reduced to at most the strain at the yield point (ε_{yield}) of the uncovered core fiber can be determined according to the following equation: ${l}_{ε} = {L}_{0} \sqrt{\left(1+\frac{{π}^{2} {ρ}_{0}^{2} {D}_{0}^{2}}{4}\right) {ε}_{max}^{2} + \left(2-{π}^{2}{ρ}_{0}^{2}{D}_{0}d-{π}^{2}{ρ}_{0}^{2}{D}_{0}^{2}\right) {ε}_{max} + \left(1+{π}^{2}{ρ}_{0}^{2}{\left({D}_{0}+d\right)}^{2}\right)}$ wherein L₀ is the length of the core fiber in the unstretched state, D₀ is the diameter of the core fiber in the unstretched state, ρ₀ is the density of entwining in the unstretched state, d is the diameter of the covering yarn, and εₘₐₓ is the strain of the core fiber at its yield point.

The covering yarn may be wound around the core fiber as single or double, covering with S- or Z-directional twists. The twist density is preferably in a range of 750 to 3000 twists per meter.

The yield point is the point on a stress-strain curve that indicates the limit of elastic behavior. Thus, the engineering strain at the yield point (ε_{yield}) is the strain (elongation) the core fiber can sustain without being permanently deformed. The yield point is a material characteristic value and can be determined according to ISO 527.

### DEATILED DESCRIPTION OF THE INVENTION

Preferably, the semi-crystalline core fiber is selected from shape-memory polymers selected from the group of polycaprolactone, poly[ethylene-co-vinyl acetate] (PEVA), poly(ethylene-1-octene), polycyclooctene containing trans-polyocentamer (PCO/TOR), poly[ethylene-co-ethyl acrylate-co-maleic anhydride] (PEEAMA), poly[ethylene-co-(methyl acrylate)-co-(glycidyl methacrylate)] (PEMAGMA), perfluorosulphonic acid ionomer (PFSA), amorphous multi block cycloaliphatic polyetherurethane (PEU) consisting of poly(tetramethylene glycol) (PTMEG), 1,4 butanediol (1,4-BD) and methylene bis(p-cyclohexyl isocyanate) (H12MDI), most preferably the semi-crystalline core fiber is of a poly[ethylene-co-vinyl acetate] (PEVA) polymer.

In an embodiment of the invention, the polymers are optionally present as a blend, wherein the content of each polymer in the blend is at least 10 wt%.

In another embodiment, the hard segment content such as (H₁₂MDI)/(1,4-BD), polyethylene co-monomer content, trans-double-bond content may preferably vary between 40% and 95% in the polymers.

The vinyl acetate in the poly[ethylene-co-vinyl acetate] polymer may preferably vary between 5% and 50% of the total weight of the polymer. In an embodiment of the invention, the poly[ethylene-co-vinyl acetate] polymer comprises a cross-linker such as triallyl isocyanorate (TAIC) and/or an initiator such as benzophenone (BP). Preferably, the amount of cross-linking agent and initiator in the poly[ethylene-co-vinyl acetate] polymer ranges from 0.5% to 5.0% by weight, such as from 1.0% to 2.0% by weight.

The nature of the covering yarn ranges from yarns of natural fibers, such as cotton, wool, etc., to semi-synthetic or synthetic yarns, such as viscose, acrylic, nylon, polyester, etc.

The diameter ratio between the covering yarn and core fiber may preferably range from 1:1 to 1:20.

The covering yarn may be a multifilament or a monofilament yarn. However, monofilament yarns are prefereed.

Preferably, the diameter of the core fiber in the cSMPF lies within 50-500 pm.

In another aspect, the present invention relates to a method for manufacturing the covered shape-memory polymeric fiber (cSMPF). The method includes the steps of extruding a core fiber of a poly[ethylene-co-vinyl acetate] polymer, optionally together with a cross-linker or cross-linking agent, optionally curing the extruded fibers for covalent cross-linking, preferably by applying radiation such as UV, beta or gamma radiation, and winding a covering yarn around the core fiber. Alternatively cross-linking can be performed by heating to temperatures below melting temperature of specific polymer defined by ISO 11357, while stretching can be performed up to 10 times comparing to unstretched extruded fiber.

In another aspect, the present invention relates to a use of the covered shape-memory polymeric fiber (cSMPF). The cSMPF can be used for example for compression garments, orthopedic bandages, orthoses, posture correction garments, push-up garments, corsets and corsages, and sports garments.

In the following, the invention will be described in detail by referring to exemplary embodiments that are accompanied by figures, in which:
- Fig. 1: shows a schematic view of covered shape-memory polymeric fiber (cSMPF) according to the present invention,
- Fig. 2A: shows a schematic view of the covered shape-memory polymeric fiber (cSMPF) according to the present invention in a unstreteched state and
- Fig. 2B: shows a schematic view of the covered shape-memory polymeric fiber (cSMPF) according to the present invention in a streteched state.

Figure 1 illustrates an exemplary embodiment of a covered shape-memory polymeric fiber (cSMPF) having a core fiber 10 and a substantially unstretchable covering yarn 20 wound around the core fiber 10. The covering yarn 20 is wound around the core fiber 10 in a manner that the maximum engineering strain (εₘₐₓ) of the core fiber 10 is reduced to at most the strain at the yield point (ε_{yield}) of the uncovered core fiber 10.

The present invention defines a cSMPF structure, which has its purpose to prevent overstretching of the core fiber 10, causing its irreversible plastic deformation and deterioration of mechanical and shape-memory properties as well as shape.

The expression "substantially unstretchable" means that the covering yarn is stiffer in relation to the core fiber. This ratio can be quantified with Young's modulus. Young's modulus is a mechanical property that measures the compressive stiffness of a solid material when force is applied lengthwise. In an embodiment of the invention, the covering yarn has higher Young's modulus than the core fiber. In another embodiment of the invention, the Young's modulus of the covering yarn is at least twice, preferably at least three times, most preferably at least five times of the Young's modulus of the of the core fiber.

In another embodiment, the ratio of the diameter of the core fiber D₀, the diameter of the covering yarn d, and the density of entwining ρ₀ are defined in a way that at during the stretching of cSMPF exists ε_{onset,} at which stretching of covering yarn 20 onsets and the slope of tangent of a stress-strain curve increases in a leap. Other parameters required to determine the ratio of D₀, d and ρ₀ are the length of the core fiber L, the length of the covering yarn l, the distance between two loops of the twist r and the number of twists n. L₀ defines the length of the core fiber in an unstretched state and L₁ defines the length of the core fiber 10 in a stretched state. D₀ defines the diameter of the core fiber 10 in an unstretched state and D₁ defines the diameter of the core fiber 10 in a stretched state. ΔL is the length change of the core fiber 10, thus Δ*L* = *L*₁ *- L*₀ . ΔD is the diameter change of the core fiber 10, thus Δ*D* = *D*₁ - *D*₀ *.*

The engineering strain ε of the core fiber 10 can then be defined as: $ε = \frac{{L}_{1}}{{L}_{0}} - 1 = \frac{ΔL}{{L}_{0}} .$

The Poisson's rate *v* of the core fiber 10 is defined as: $ν = - \frac{\frac{ΔD}{{D}_{0}}}{\frac{ΔL}{{L}_{0}}} .$

The formula of the Poisson's rate *v* of the core fiber 10 can be rewritten as $\frac{{D}_{1}}{{D}_{0}} = 1 - ν \frac{ΔL}{{L}_{0}} = 1 - νε .$

From the formulas just defined, the following dependencies can be derived: ${D}_{1} = ε \left(1-νε\right) ,$ ${L}_{1} = {L}_{0} \left(ε+1\right) .$

The engineering strain of the covering yarn ε*ₗ* can be expressed as a function of the engineering strain of the core fiber ε: ${ε}_{l} = {ε}_{l} \left(ε\right) = \frac{{l}_{1} - {l}_{0}}{{l}_{0}} = \frac{Δl}{{l}_{0}} = \frac{{l}_{1}}{{l}_{0}} - 1 ,$
wherein *l*₁ can be defined as: ${l}_{1} = {L}_{0} \sqrt{\left(1+\frac{{π}^{2} {ρ}_{0}^{2} {D}_{0}^{2}}{4}\right) {ε}^{2} + \left(2-{π}^{2}{ρ}_{0}^{2}{D}_{0}d-{π}^{2}{ρ}_{0}^{2}{D}_{0}^{2}\right) ε + \left(1+{π}^{2}{ρ}_{0}^{2}{\left({D}_{0}+d\right)}^{2}\right)}$

This formula for the length of the covering yarn 20 in the stretched state *l*₁ can be derived as follows. First the equation for the circumference of the core fiber 10 and the covering yarn 20 is established. Since the covering yarn 20 is wound in spirals around the core fiber 10, the number of twists n is multiplied by the distance between two twists in the stretched state r₁ and added to the circumference. ${l}_{1}^{2} = {π}^{2} {n}^{2} {\left({D}_{1}+d\right)}^{2} + {r}_{1}^{2} {n}^{2}$

For n and D₁, the formulas already established above are used and instead of ${r}_{1}^{2} {n}^{2}$ the parameter ${L}_{1}^{2}$ is used. ${l}_{1}^{2} = {L}_{0}^{2} {{ρ}_{0}}^{2} {π}^{2} {\left({D}_{0}\left(1-νε\right)+d\right)}^{2} + {L}_{1}^{2}$

Now the formula obtained above is used for L₁ and the equation is brought into the form of a quadratic equation. $\begin{matrix}{l}_{1}^{2} = {L}_{0}^{2} {{ρ}_{0}}^{2} {π}^{2} \left({D}_{0}^{2}-2{D}_{0}^{2}νε+{D}_{0}^{2}{ν}^{2}{ε}^{2}+2{D}_{0}d-2{D}_{0}dνε+{d}^{2}\right) + {L}_{0}^{2} + 2 {εL}_{0}^{2} + {ε}^{2} {L}_{0}^{2} \\ = {L}_{0}^{2} \left(\left(1+{π}^{2}{ν}^{2}{{ρ}_{0}}^{2}{D}_{0}^{2}\right){ε}^{2}+\left(2-2{π}^{2}{{νρ}_{0}}^{2}{D}_{0}d-2{π}^{2}{{νρ}_{0}}^{2}{D}_{0}^{2}\right)ε+\left(1+{π}^{2}{{ρ}_{0}}^{2}{\left({D}_{0}+d\right)}^{2}\right)\right)\end{matrix}$

For the selected materials the *ε* is limited with elastic limit, which means that elongation can be considered elastic. Therefore, no major structural reorganization takes place at molecular level. From this follows that a constant volume can be assumed, so that the Poisson's ratio can be assumed as = 0.5 . This leads to the formula: $\begin{matrix}{l}_{1} = l \left(ε\right) \\ = {L}_{0} \sqrt{\left(1+\frac{{π}^{2} {{ρ}_{0}}^{2} {D}_{0}^{2}}{4}\right) {ε}^{2} + \left(2-{π}^{2}{{ρ}_{0}}^{2}{D}_{0}d-{π}^{2}{{ρ}_{0}}^{2}{D}_{0}^{2}\right) ε + \left(1+{π}^{2}{{ρ}_{0}}^{2}{\left({D}_{0}+d\right)}^{2}\right)}\end{matrix}$

For *l*₀ the following formula is obtained: $\begin{matrix}{l}_{0}^{2} = {π}^{2} {n}^{2} {\left({D}_{0}+d\right)}^{2} + {r}_{0}^{2} {n}^{2} \\ = {π}^{2} {L}_{0}^{2} {{ρ}_{0}}^{2} {\left({D}_{0}+d\right)}^{2} + {L}_{0}^{2} \\ = {L}_{0}^{2} \left({π}^{2}{{ρ}_{0}}^{2}{\left({D}_{0}+d\right)}^{2}+1\right) \\ {l}_{0} = {L}_{0} \sqrt{1 + {π}^{2} {{ρ}_{0}}^{2} {\left({D}_{0}+d\right)}^{2}}\end{matrix}$

The εₒₙₛₑₜ is defined as *ε*, at which *εₗ*(*ε*) becomes positive. $\begin{matrix}{ε}_{l} = {ε}_{l} \left(ε\right) = \frac{{l}_{1}}{{l}_{0}} - 1 \\ = \frac{\sqrt{\left(1+\frac{{π}^{2} {{ρ}_{0}}^{2} {D}_{0}^{2}}{4}\right) {ε}^{2} + \left(2-{π}^{2}{{ρ}_{0}}^{2}{D}_{0}d-{π}^{2}{{ρ}_{0}}^{2}{D}_{0}^{2}\right) ε + \left(1+{π}^{2}{{ρ}_{0}}^{2}{\left({D}_{0}+d\right)}^{2}\right)}}{\sqrt{\left(1+{π}^{2}{{ρ}_{0}}^{2}{\left({D}_{0}+d\right)}^{2}\right)}} - 1 \\ = \sqrt{1 + \frac{2 - {π}^{2} {{ρ}_{0}}^{2} {D}_{0} d - {π}^{2} {{ρ}_{0}}^{2} {D}_{0}^{2}}{1 + {π}^{2} {{ρ}_{0}}^{2} {\left({D}_{0}+d\right)}^{2}} ε + \frac{1 + {π}^{2} {{ρ}_{0}}^{2} {D}_{0}^{2} / 4}{1 + {π}^{2} {{ρ}_{0}}^{2} {\left({D}_{0}+d\right)}^{2}} {ε}^{2}} - 1\end{matrix}$

By following the ratio between *D*₀*, d* and *ρ*₀ the stretching of the core fiber 10 can be avoided by selecting *D*₀, *d* and *ρ*₀, so that Δ*l* and thus the engineering strain of the covering yarn *εₗ*(*ε*) becomes positive only when the maximum engineering strain (εₘₐₓ) of the core shape-memory fiber 10 is passed.

Thus the covering yarn 20 is wound around the core fiber 10 in a manner that after stretching to a defined engineering strain (εₘₐₓ), the covering fiber will be so deformed that further stretching of cSMPF will cause axial stretching of the covering yarn. If the core fiber 10 is stretched at a temperature between glass transition and melting temperature defined by ISO 11357 up to the engineering strain (εₘₐₓ) and released, will recover the residual deformation, if heated to a temperature between 25 °C and melting temperature defined by ISO 11357.

Figure 2A and 2B illustrate exemplary embodiments of two states of a covered shape-memory polymeric fiber. In both states the covered shape-memory polymeric fiber has a core fiber 10 and a substantially unstretchable covering yarn 20 wound around the core fiber 10. In Figure 2A the core fiber 10 is in a unstretched state. Figure 2B shows the core fiber 10 in a stretched state. The change in coils/twists spacing of the covering yarn 20 upon mechanical deformation of the core fiber 10 during programming (from Figure 2A to Figure 2B) and recovery (from Figure 2B to Figure 2A) can be seen. Stretching (elongation) of the core fiber 10 having the covering yarn 20 wound around it causes the pitch, i.e. the distance between two loops of the twist, of the covering yarn 20 around the core fiber 10 to increase from r₀ to r₁, whereby the density of entwining (ρ₁) decreases.

### EXAMPLE

The polymers in the core fiber or their blends can be cross-linked with covalent bonds, ionic interactions or crystallites. Covalently cross-linked polymer networks have a gel content of 60 -100% according to ASTM D2765 or ISO 10147. The gel content (G) of cross-linked core fibers was estimated by extraction in solvents such as toluene or xylene at constant temperature ≤110°C. Extraction time was 24 h, with another 24 h for solvent evaporation in vacuum oven at 45 °C. G was calculated from the isolated weight *m*ᵢₛₒ of the sample and the dry weight *m*_{d} after extraction using the equation below. However, non-extracted fibers were used for covering and for investigations such as thermo-mechanical and shape-memory properties $G = \frac{{m}_{d}}{{m}_{iso}} ∗ 100 %$

Semi-crystalline cross-linked poly[ethylene-co-vinyl acetate] (cPEVA) fibers were covered with single or double covering of yarn with 750 to 3000 twists per meter. The number of twists were adjusted to allow certain deformation but to reduce the maximum engineering strain (εₘₐₓ) of the core shape-memory fiber to at most the strain at the yield point (ε_{yield}) of the uncovered core fiber.

The effect of the twist density and angle of the covering yarn on the stretchability during programming and recovery of the SMP covered yarns was evaluated.

The mechanical properties of the covered and non-covered shape-memory fibers were tested by tensile testing at room as well as at elevated temperatures (above and within the broad melting transition ranges). These tensile tests were conducted on a Zwick/Roell machine Z005 (Zwick, Ulm, Germany) equipped with a thermo-chamber and temperature controller (Eurotherm Regler, Limburg, Germany) with a strain rate of 5 mm·min⁻¹. The selected temperature for such measurements were 25°C, 37°C, 40°C, 50°C, 60°C, 70°C, 80°C and 90°C. Elastic modulus (*E*), elongation at break (*ε*_{break}) and stress at break (*σ*_{break}) were obtained and analyzed.

Similarly, the shape-memory characteristic of the fibers were evaluated on a Zwick/Roell machine Z005 (Zwick, Ulm, Germany) equipped with a thermo-chamber and temperature controller (Eurotherm Regler, Limburg, Germany). Each shape-memory cycle within one experiment consisted of an initial programming step followed by a recovery step under stress-free conditions with heating and cooling rates ≤ 10°C·min⁻¹. Each shape-memory test consisted of at least three cycles. A single step programming procedure was applied, where the sample was stretched with a rate of ≤ 10 mm·min⁻¹ to a certain programming strain (*ε*_{prog}) at programming temperature (*T*_{prog}) followed by an equilibration time of ≤ 10 min and cooling below crystallization temperature (≤25 °C) under constant strain. After another ≤10 min equilibration time, the stress was released at this lower temperature and the sample was reheated to recovery temperature (*T*_{rec}). A constant force of ≤0.1N was applied on the specimen during recovery cycle. The *T*_{rec} can be anywhere within the melting range of the polymer and can identical to *T*_{prog}. The shape-fixity ratios and recovery ratio were calculated from second and third cycles and the results were analyzed.

The shape fixity (R_{f}) and shape recovery (Rᵣ) in a cycle (N) can be calculated from applied deformation (εₘ) during programming, fixed strain in the temporary shape (εᵤ) after removing stress in the programming step and recovered strain (εₚ) in the recovery cycle using following equations. ${R}_{f} \left(N\right) = \frac{{ε}_{u} \left(N\right)}{{ε}_{m}} \times 100$ ${R}_{r} \left(N\right) = \frac{{ε}_{u} \left(N\right) - {ε}_{p} \left(N\right)}{{ε}_{u} \left(N-1\right) - {ε}_{p} \left(N-1\right)} \times 100$

The shape-recovery ratio for the covered fibers were ≥95% In order to ensure and evaluate long term shape-memory capability of these fibers, a test with ~100 shape-memory cycles was performed which showed identical results for shape-recovery and lower shape fixity ratios over the course of 100 cycles. For practical reasons and in order to reduce the time for one cycle, the heating and cooling rates were 10°C·min⁻¹ here and equilibration times were reduced to 1 min.

## Claims

1. Covered shape-memory polymeric fiber (cSMPF) having a core fiber, and a substantially unstretchable covering yarn wound around the core fiber in a manner that the maximum engineering strain of the core fiber is reduced to at most the strain at the yield point of the uncovered core fiber.

2. The covered shape-memory polymeric fiber of claim 1 wherein the core fiber is selected from shape-memory polymers selected from the group of polycaprolactone, poly[ethylene-co-vinyl acetate] (PEVA), poly(ethylene-1-octene), polycyclooctene containing trans-polyocentamer (PCO/TOR), poly[ethylene-co-ethyl acrylate-co-maleic anhydride] (PEEAMA), poly[ethylene-co-(methyl acrylate)-co-(glycidyl methacrylate)] (PEMAGMA), perfluorosulphonic acid ionomer (PFSA), amorphous multi block cycloaliphatic polyetherurethane (PEU) consisting of poly(tetramethylene glycol) (PTMEG), 1,4 butanediol (1,4-BD) and methylene bis(p-cyclohexyl isocyanate) (H12MDI).

3. The covered shape-memory polymeric fiber of claim 2 wherein the vinyl acetate content in the poly[ethylene-co-vinyl acetate] polymer is between 5% and 50% of the total weight of the polymer.

4. The covered shape-memory polymeric fiber according to any one of claims 2 and 3 wherein the poly[ethylene-co-vinyl acetate] polymer comprises a cross-linker and/or an initiator.

5. The covered shape-memory polymeric fiber according to claim 4 wherein the amount of cross-linking agent and initiator in the poly[ethylene-co-vinyl acetate] polymer ranges from 0.5% to 5.0% by weight.

6. The covered shape-memory polymeric fiber according to any one of claims 4 and 5 wherein the cross-linker is triallyl isocyanorate (TAIC).

7. The covered shape-memory polymeric fiber according to any one of claims 4 to 6 wherein the amount of cross-linking agent and initiator in the poly[ethylene-co-vinyl acetate] polymer ranges from 1.0% to 2.0% by weight.

8. The covered shape-memory polymeric fiber according to any one of claims 4 to 7 wherein the cross-linking agent is benzophenone (BP).

9. The covered shape-memory polymeric fiber according to any one of the previous claims wherein the covering yarn is selected from cotton, wool, silk, linen, viscose, acrylic, nylon and polyester.

10. The covered shape-memory polymeric fiber according to any one of the previous claims wherein the covering yarn is wound around the core fiber as single or double covering with S or Z direction twists.

11. The covered shape-memory polymeric fiber according to any one of the previous claims wherein the diameter ratio between the covering yarn and core fiber lies preferably within 1:1 to 1:20.

12. The covered shape-memory polymeric fiber according to any one of the previous claims wherein the diameter of the core fiber lies within 50-500 pm.

13. The covered shape-memory polymeric fiber according to any one of the previous claims wherein the covering yarn is a monofilament yarn.

14. A method for producing the covered shape-memory polymeric fiber as claimed in any one of the previous claims including the steps of extruding a core fiber of a poly[ethylene-co-vinyl acetate] polymer, optionally together with a cross-linker or cross-linking agent, optionally curing the extruded fibers for covalent cross-linking and winding a covering yarn around the core fiber.

15. The method of claim 14 wherein the curing takes place under UV, beta or gamma radiation.

16. A use of the covered shape-memory polymeric fiber as claimed in any one of claims 1 to 13 for compression garments, orthopedic bandages, orthoses, posture correction garments, push-up garments, corsets and corsages, and sports garments.
